

May 31, 1927.

1,630,267

A. S. KREBS

METHOD AND APPARATUS FOR QUENCHING LITHOPONE

Filed June 29, 1923

Fig. 1.



Fig. 2.



Inventor:  
A. Sonnino Krebs.

by Francis C. Lasker  
his Attorney

Patented May 31, 1927.

1,630,267

# UNITED STATES PATENT OFFICE.

AUGUST SONNIN KREBS, OF WILMINGTON, DELAWARE, ASSIGNOR TO THE KREBS PIGMENT & CHEMICAL COMPANY, OF NEWPORT, DELAWARE, A CORPORATION OF DELAWARE.

## METHOD AND APPARATUS FOR QUENCHING LITHOPONE.

Application filed June 29, 1923. Serial No. 648,431.

My invention relates to the manufacture of lithopone and particularly to the quenching of the hot lithopone as it comes from the calcining furnace in which crude lithopone 5 is heated in the well known process of manufacturing lithopone. The object of my invention is to provide a better method of quenching the hot lithopone with a special view to the convenient handling of the 10 material, the avoidance of the formation of an objectionable amount of steam, economy in the use of quenching water and the obtaining of a better and more uniform mixture of the lithopone than has heretofore 15 been practicable.

The nature of my improved method, and the apparatus which I have devised for practising it, will be best understood as described in connection with the drawings 20 which illustrate an apparatus designed for use in accordance with my method and in which

Figure 1 is a plan view showing a number of calcining furnaces and provisions 25 for quenching and mixing the lithopone in accordance with my invention, and

Figure 2 is a sectional elevation on line 2—2 of Fig. 1.

A, A, etc. are furnaces for heating the 30 muffles. B, B, etc. represent rotary tube muffles of the general character described in my co-pending application for Letters Patent filed April 14, 1923, Serial No. 632,045. To the tubes B which extend 35 through openings A' A<sup>2</sup>, in the furnace are secured extensions B', B<sup>2</sup>, having tires or rims C, C', secured to them which rest on rollers G, G. The extension B has also a sprocket wheel D secured to it and the extension B' is covered with a non conducting 40 packing E. F is a restricted delivery spout at the end of the muffle. H is a hopper into which the crude lithopone is charged and from which the lithopone is 45 fed into the muffle through conduit H' by a screw conveyer I driven through a sprocket I', chain K and sprocket J' attached to driving shaft J. To shaft J is also attached a sprocket J<sup>2</sup> connected to rotate the muffle 50 through chain K' and sprocket D. The driving shaft also actuates a rapper indicated at L and fully described in my aforesaid application.

M is a launder or pipe through which a

constant flow of water is maintained, flowing, as shown, from a reservoir M' fed by pipe N and through pipe M to tank O. M<sup>2</sup>, M<sup>2</sup>, etc. are conduits registering with delivery spouts F and opening into pipe M. P and P' are thermocouples by which the temperature of the furnace and muffle can be ascertained.

In operation the muffle furnaces are in continuous operation and deliver the calcined lithopone in a uniform and fine stream through the spouts F and conduits M<sup>2</sup> into the launder M. Through this launder a continuous stream of water is maintained of sufficient quantity to quench the streams of hot lithopone entering the launder without the formation of any considerable amount of steam. The lithopone is transported through the launder to the settling tank O and where, as in the illustration, a number of calcining furnaces are simultaneously delivering lithopone into the launder and tank, the product of all these furnaces is thoroughly mixed together in the launder and tank with the result that a better averaging up and mixture of the different furnace products is effected than has heretofore 70 been practicable. Indeed, by my method I obtain a better mixture and more uniform quantity of lithopone than has heretofore 75 been practicable by any of the expedients used in the treatment of the furnace product with which I am familiar.

Having now described my invention, what I claim as new and desire to secure by Letters Patent is:

1. The method of quenching calcined lithopone which consists in feeding the hot lithopone in a continuous fine stream into a running stream of water and continuously conveying the quenched lithopone to a settling tank by means of said running stream.

2. The method of quenching and mixing calcined lithopone produced in two or more calcining furnaces which consists in simultaneously feeding the hot lithopone in continuous fine streams from the furnaces into a body of quenching water.

3. The method of quenching and mixing calcined lithopone produced in two or more calcining furnaces which consists in simultaneously feeding the hot lithopone in continuous fine streams from the furnaces into a running stream of water.

4. Apparatus for quenching lithopone comprising in combination one or more continuously operating calcining furnaces having provision for a continuous delivery of hot calcined lithopone, a running water conduit of narrow cross section adapted to maintain the running water in constant uniform motion arranged to directly receive, quench and transport the lithopone continuously delivered to it from the furnace or

furnaces, and a settling tank at the delivery end of the conduit.

5. Apparatus for quenching lithopone comprising in combination two or more continuously operating calcining furnaces having provision for the continuous delivery of hot calcined lithopone, a water conduit arranged to receive the lithopone from the furnaces and a settling tank.

A. SONNIN KREBS.